

## [54] PROCESS FOR PRODUCTION OF METAL-PLATED FIBERS

2,425,214 8/1947 Voelker et al. .... 118/315  
3,663,242 5/1972 Gulla ..... 117/47 A

[75] Inventors: Minoru Maeawa; Morioka, Hiroka, both of Okayama, Japan

Primary Examiner—William D. Martin

[73] Assignee: Kuraray Co., Ltd., Kurashiki, Okayama prefecture, Japan

Assistant Examiner—Janyce A. Bell

[22] Filed: Oct. 10, 1972

Attorney, Agent, or Firm—Sherman &amp; Shalloway

[21] Appl. No.: 296,021

## [30] Foreign Application Priority Data

Oct. 14, 1971 Japan ..... 46-81135

[52] U.S. Cl. .... 117/47 A, 8/115.6, 117/105.3, 117/105.4, 117/138.8 PV, 117/160 R, 118/305, 118/307, 118/315, 118/320

[51] Int. Cl. .... B44d 1/092

[58] Field of Search ..... 117/47 A, 160 R, 105.4, 117/105.3, 138.8 PV; 118/307, 320, 315, 305; 8/115.6

## [56] References Cited

## UNITED STATES PATENTS

2,410,626 11/1946 Boudreau ..... 118/315

## [57] ABSTRACT

A process for the production of metal-plated fibers by electrolessly plating pre-treated fibers, which comprises reeling the fibers into hanks, hanging the fibers in the hank form on a rotary cylinder having projection holes to suspend the fibers in the air, allowing the fibers to move rotatively around the cylinder by rotation of the cylinder, projecting a plating solution at a rate of 5 to 50 cm/sec from said projection holes against the rotatively moving fibers and thereby effecting the electroless plating of the fibers.

6 Claims, 3 Drawing Figures



PATENTED FEB 4 1975

3,864,148

Fig. 1



Fig. 2



Fig. 3



## PROCESS FOR PRODUCTION OF METAL-PLATED FIBERS

This invention relates to a process for the production of metal-plated fibers by the electroless plating method.

In conventional methods of the electroless plating of fibers, fibers which have been subjected to such pre-treatments as deoiling, etching, activation and the like are generally dipped in electroless plating solutions containing metallic ions, reducing agents, complexing agents, hydrogen ion-adjusting agents, stabilizers and other additives. In the case of fibers the surface area is much greater than in the case of molded articles of plastics having the same weight, and in threads the distances between individual fibers are very short and they are very close to one another. Further, in the electroless plating of threads, fine bubbles of hydrogen and other gases are generated from the fiber surfaces as the plating reaction advances. For these reasons, penetration of a plating solution into fibers is inhibited and unevenness of plating is brought about between the surface layer and inner layer of a thread. Accordingly, in conventional methods of the electroless plating of fibers, it is impossible to obtain metal-plated fibers having uniform plating layers.

It is therefore a primary object of this invention to provide an economical process which can overcome such defects of the conventional methods and can provide metal-plated fibers having uniform plating layers.

In accordance with this invention, there is provided a process for the production of metal-plated fibers by electrolessly plating pre-treated fibers, which comprises reeling the fibers into hanks, hanging the fibers in the hank form on a rotary cylinder having projection holes to suspend the fibers in the air, allowing the fibers to move rotatively around the cylinder by rotation of the cylinder, projecting a plating solution from said projection holes at a rate of 5 to 50 cm/sec against the rotatively moving fibers and thereby effecting the electroless plating of the fibers.

This invention will now be detailed by reference to the accompanying drawings in which:

FIG. 1 is a diagram illustrating one embodiment of apparatus for use in the practice of the electroless plating according to this invention;

FIG. 2 is a sectional view illustrating the state in the fibers of the hank form being hung on the rotary cylinder of the apparatus illustrated in FIG. 1; and

FIG. 3 is a diagram illustrating the state where the fibers in the hank form to be subjected to the electroless plating treatment are tied by lea threads and divided into several portions.

Any chemical fibers such as polyamide fibers, polyester fibers, polyolefin fibers, polyvinyl alcohol fibers, polyacrylonitrile fibers, acetate fibers and rayon fibers and natural fibers such as cotton and wool fibers may be electrolessly plated according to this invention. Among these fibers, polyvinyl alcohol fibers are most preferably treated according to the process of this invention, because polyvinyl alcohol fibers have the property that metal-plated fibers excellent in durability of adherence between the plating layer and fibers can be obtained, even if the etching pre-treatment is not effected. In the case of other fibers, the etching pre-treatment is indispensable because without the etching pre-treatment the adherence durability is much low-

ered and it is impossible to obtain metal-plated fibers of practical value. Further, as is illustrated in the Examples given hereinbelow, in the case of polyvinyl alcohol fibers the surprising result is obtained that the adherence durability of metal-plated fibers derived from polyvinyl alcohol fibers which have not been subjected to the etching pre-treatment is superior to the adherence durability of metal-plated fibers derived from other fibers which have been subjected to the etching pre-treatment. Polyacrylonitrile fibers are most preferred among fibers other than polyvinyl alcohol fibers, but omission of the etching pre-treatment is not permissible in polyacrylonitrile fibers.

The fibers to be metal-plated according to the process of this invention may take any form. For instance, they may be a monofilament, multi-filament yarn, spun yarn, split yarn, tape yarn, cord, tape, etc. In the instant specification and claims, the term "fiber" or "fibers" is used to mean all of these fibrous articles inclusively.

The process of this invention will now be explained by referring, for convenience's sake, to an embodiment where multi-filament yarn is treated as a typical instance of such fibrous articles.

Methods for the electroless plating of fibers and molded articles of plastics have been known in the art. In general, articles to be treated are subjected successively to such pre-treatments as deoiling, etching and activation, and then they are dipped in an electroless plating solution to effect the electroless plating. In this invention, these pre-treatments may be conducted according to customary procedures and no modification is necessary. More specifically, in the deoiling treatment fibers are treated with a neutral detergent or warm water to remove oils applied to fiber surfaces.

After this deoiling treatment, the etching treatment is conducted in the case of other fibers than polyvinyl alcohol fibers. For instance, polyester and polyacrylonitrile fibers are treated with etching agents such as alkali metal hydroxides and polyolefin and polyamide fibers are treated with such etching agents as solutions of the chromic acid-sulfuric acid type. Other fibers are subjected to the etching treatment with use of appropriate etching agents such as alkaline substances, chromic acid, etc. As described hereinabove, this etching treatment can be omitted in the case of polyvinyl alcohol fibers, which results in an industrial advantage of reduction of the manufacturing cost. After the etching treatment, the activation treatment is conducted. This activation treatment is also accomplished according to customary procedures. For instance, fibers are activated by a method comprising treating fibers with a hydrochloric aqueous solution of stannous chloride, washing the fibers with water, treating the fibers with a hydrochloric aqueous solution of palladium chloride, and washing the fibers with water to remove unreacted palladium chloride remaining on fiber surfaces or in voids formed among the fibers. Fibers may be subjected to these pre-treatments in the form of cheese, cone or hank, but it is preferred that these pre-treatments are effected on fibers in the hank form.

Fibers which have been subjected to these pre-treatments are then the electroless plated. As will be apparent from the description given below, the electroless plating process of this invention is unique and different from electroless plating techniques heretofore adopted in the art. Furthermore, the electroless plating process of this invention can give a plating layer which

is superior in its uniformity and evenness over plating layers formed by the conventional electroless plating techniques.

In FIGS. 1 and 2, fibers 1 in the hank form ready to be plated, which have passed through the steps of the abovementioned pre-treatments, are hung on a rotary cylinder 5 in a uniform thickness with no overlapping of hanks. This cylinder 5 is driven by a motor 10, and the fibers 1 are moved rotatively around the rotary cylinder 5 by rotation thereof. The rotary cylinder 5 is provided with partition plates 2 for preventing the overlapping of hanks during the operation and with forwarding plates 3 for conducting the rotary movement of the hanks smoothly. Projecting holes 4 are mounted on the rotary cylinder 5 to project a plating solution against the fibers 1. In FIG. 1, a plating solution 7 contained in a plating solution tank 11 is fed to the cylinder 5 by means of a pump 8 after its temperature has been adjusted to a prescribed level by a heating or cooling device, and the solution 7 is projected against the fibers 1 of the hank form through projection holes 4. The adjustment in the feed rate of the plating solution and the agitation of the plating solution are accomplished by means of a valve 9. Thus, the fibers 1 in the hank form are contacted with the plating solution projected through the projection holes 4 and the electroless plating is accomplished. The plating solution flows downwardly along the fibers in the hank form suspended in the air, and is returned to the tank 11. In this treatment, in order to obtain a uniform plating layer, it is important that the lower ends of the hanks of the fibers 1 hung on the cylinder 5 do not contact the liquid face of the plating solution contained in the tank 11. It is desirable that the system for circulation (i.e. tank or cylinder) of the plating solution be lined with glass or plastic so as to prevent occurrence of the plating reaction by contact with the plating solution. Occurrence of the undesired plating of the circulation system may also be prevented if the system is constructed of stainless steel.

The most important feature of the process of this invention reside, as described above, in that the electroless plating is effected while projecting a plating solution against fibers hung (in the form of hanks) on the rotary cylinder which is provided with plating solution-projecting holes. In this electroless treatment, it is important that the fibers in the hank form are hung on the rotary cylinder uniformly in either the lateral direction or the thickness direction, and the overlapping of the hanks of fibers or unequal distribution of the fibers hung on the rotary cylinder must be avoided as much as possible. For this purpose, partition plates 2 are mounted on the rotary cylinder 5. The uniform hanging of the fiber hanks can be effectively attained by tying the hanks with the use of lea threads and dividing each hank into several portions, which feature is illustrated in FIG. 3. The plating solution is then projected through the projection holes against the fibers hung in the form of hanks uniformly on the rotary cylinder. By adopting such unique electroless plating means according to this invention, it is made possible for the plating solution to penetrate easily even into interiors of the fiber assembly, and therefore, metal-plated fibers having a uniform plating layer can be obtained.

In this invention it is necessary that the plating solution should be projected at a rate ranging from 5 to 50 cm/sec, preferably from 15 to 35 cm/sec. At a projection rate of less than 5 cm/sec, the penetration of the

plating solution is prevented by fine bubbles formed with the advance of the plating reaction, which results in occurrence of unevenness of the plating layer. At a projection rate exceeding 50 cm/sec, although a uniform plating layer is obtainable, the hanks become greatly disordered and are difficult to reel. Moreover, when the plating solution is projected at a rate exceeding 50 cm/sec, the plating layers formed on the fibers tend to peel off easily, the reason for which is unknown. 10 Accordingly, too high a projection rate is not preferred. In view of the durability of adherence between the plating layer and the fibers, the flexibility of the resulting plated fibers, and the effects on the resulting plated fibers when used for antistatic purposes, it is desired that each individual filament has a denier of from 0.1 to 15, and especially from 1 to 6. In the case of fibers having a filament denier of less than 0.1 good durability of adherence can be attained between the plating and the fibers, however the flexibility inherent in the fibers is lost when the metal is plated to a thickness of about 1  $\mu$ , and the surface area per unit weight is increased, resulting in an economic disadvantage. In the case of fibers having a filament denier exceeding 15, the durability of adherence between the plating layer and the fibers is reduced because of swelling and expansion of the fibers brought about during the plating step or shrinkage of the fibers caused during the drying or cooling step. Furthermore, cracks are readily formed in the metal plating layer by mechanical deformation or the like. Additionally, plated fibers derived from fibers having a filament denier exceeding 15 exhibit low anti-static activity. For these reasons, the use of fibers having a filament denier exceeding 15 is not preferred.

35 Where the electroless plating process of this invention is applied to monofilaments, cords and the like, it is preferred that the total denier of the fibers to be plated is more than 20. The upper limit of the total denier is not particularly critical and even fibers having a total denier of about 1,000 can be conveniently treated according to the electroless plating process of this invention.

40 The size of the hank to be used in this invention is determined appropriately depending on the amount of 45 the fiber treated, of the fiber, the form of the fiber, the size of the electroless plating apparatus and other factors, but it is generally preferred that a hank has a weight of from 30 to 500 g per 1.5 m circle. In case the hank has a weight of less than 30 g per 1.5 m circle, it 50 takes a long time to effect the reeling and the use of such hank is not economical. Use of a hank having a weight of greater than 500 g per 1.5 m circle is also undesired because the penetration of the plating solution into the hank fibers is insufficient.

55 It is preferred that the lea thread to be used for tying the hanks exhibits a shrinkage not exceeding 5 percent during the plating step. When the lea thread shrinks by more than 5 percent during the plating step, the part tied by the lea thread undergoes contraction and penetration of the plating solution into the fibers of this part is insufficient, with the result that unevenness is brought about in the resulting plating layer.

60 It is desired that the hank be divided into 3 to 6 portions per 1.5 m with the lea thread. In case the number of leas is less than 3 per 1.5 m, the hanks become disordered during the plating step and consequently, the hanks are difficult to reel. Penetration of the plating so-

lution is insufficient when the number of leas exceeds 6 per 1.5 m.

In a preferable embodiment of this invention, one hank of fibers is hung on each section of the rotary cylinder such section being partitioned by two partition plates. The distance between two adjoining partition plates is varied depending on the size of the hank, but it is generally preferable that the distance be within a range of from 5 to 10 cm. A preferable amount of fibers hung on one section partitioned by the two adjoining partition plates is within a range of from 30 to 500 g, especially 50 to 200 g.

The rate of rotation of the fibers hung in the hank form on the rotary cylinder is not critical but a rotation rate of about 9 to about 18 m/min is usually adopted. The rotation direction may be reversed at suitable intervals, for instance, every two minutes.

It is preferred that the projection holes for projecting a plating solution have a diameter of from 2 to 5 mm and that such projection holes are distributed on the rotary cylinder to such an extent that 25 to 150 projection holes are present per 100 cm<sup>2</sup> of the surface of the rotary cylinder. In case the number of projection holes is less than 25 per 100 cm<sup>2</sup>, the thickness of the plating layer differs in the outer and interior portions of the plated thread and it is difficult to obtain metal-plated fibers having a uniform plating layer. In case the number of projection holes is more than 150 per 100 cm<sup>2</sup>, it is difficult to maintain the constant flow rate of the plating solution at a prescribed level.

It is preferred that the plating reaction is carried out at a temperature ranging from 40° to 100°C. The reaction time varies depending on the amount of fibers to be treated and the intended amount of the metal to be plated on the fibers, but generally, the reaction is conducted for from 5 to 30 minutes.

In this invention it is possible to use a conventional solution for electroless plating which contains, in addition to ions of a metal to be plated on the fibers, a reducing agent, a complexing agent, a hydrogen ion-adjusting agent and other additives. The plating solution may further contain a stabilizer according to need. As the metal to be plated on fibers, there may be mentioned nickel, copper, cobalt, chromuim, tin, etc. The metals be used singly or in the form of mixtures of two or more (for instance, a mixture of nickel and cobalt). In view of the stability of the plating solution and the rate of the plating reaction, the use of nickel and copper, especially nickel, is preferred. In this invention, an electrolytic plating may be formed on the resulting electroless plating layer, if desired.

In a very preferable embodiment of this invention, the plating reaction is conducted by employing a plating solution containing at least one stabilizer selected from: guanidines such as diphenyl guanidine and di-ortho-tolyl guanidine; thiourea derivatives such as thiocarbanilide; imidazoline derivatives such as 2-mercaptoimidazoline; dithiocarbamic acid salts such as sodium dimethyldithiocarbamate and sodium dibutylidithiocarbamate; thiurams such as tetramethyl thiuram disulfide; thiiazoles such as mercaptobenzothiazole; and imidazoles such as mercaptobenzimidazole. It is possible to conduct the electroless plating process of this invention by employing a plating solution free of such stabilizer, but that causes the undesired phenomenon of blacking of the plating solution in a short time from initiation of the plating reaction.

Once blacking occurs in the plating solution, the plating reaction does not proceed on the material to be plated and a black substance is deposited on the plating surface, which results in degradation of the appearance of the product. Accordingly, in this invention it is preferable to employ a plating solution containing a stabilizer such as mentioned above. It is considered that this undesired phenomenon of blacking is due to the self-decomposition of the plating solution, and it has been known to avoid occurrence of this phenomenon by incorporation of a stabilizer such as sodium thiosulfate. However, known stabilizers lose their stabilizing activity in a relatively short time when incorporated in a plating solution maintained at high temperatures, and they cannot be used for a long time or continuously. By contrast, the specific stabilizers exemplified above are advantageous over known stabilizers in that their stabilizing activity undergoes no change even if they are used at high temperatures for a long time. The specific stabilizer to be used in this invention is incorporated preferably in an amount of 0.5 to 20 mg per liter of the plating solution. Among the stabilizers exemplified above, mercapto group-containing stabilizers such as mercaptobenzimidazole, mercaptobenzthiazole and 2-mercaptoimidazoline exhibit particularly great stabilizing effects. Since many of these stabilizers are difficultly soluble in the plating solution when it is necessary to incorporate them in great quantities, it is preferred that these stabilizers are used in the form of an aqueous solution of caustic alkali, e.g., an aqueous solution of sodium hydroxide of 0.05 - 1 N.

The metal-plated fibers obtained according to the process of this invention usually have a metal plating layer with a thickness ranging from 0.01 to 15 microns, and preferably from 0.05 to 2.0 microns.

The metal-plated fibers obtained according to the process of this invention are superior to metal-plated fibers formed by conventional methods where fibers to be plated are dipped in plating solutions in that the thickness of the plating layer is highly uniform and hence, the deviation of the electric resistance in the longitudinal direction is very small.

The metal-plated fibers, as they are or after incorporation with unplated fibers, are used in the form of knitted fabrics, woven fabrics, non-woven fabrics, cords or tapes, and as electric heaters, protective suits for high voltage linemen, electromagnetic shieldings, and the like. Further, when they are incorporated in fibrous and plastic products in which static charges are readily generated and accumulated, an antistatic effect is attained in these products.

This invention will now be illustrated more detailedly by reference to Examples, but it is of course not limited by these Examples.

Values of the thickness of the plating layer of the metal plated fibers are those calculated by the weight method or microscope method. The values measured by the two methods agree with each other quite well.

#### EXAMPLE 1

A hank of a circle of 1.5 m was prepared from 100 g of filaments of 250 denier/36 filaments (which will be abbreviated as "250 dr/36 f" below) having a twist number of 150 turns per meter and composed of a polyvinyl alcohol having a degree of formalization of 20 mole percent (sold under the trademark "Vinylon"), and the hank was tied with a lea thread and divided into

5 portions. Ten hanks were prepared in the above manner and subjected to the deoiling treatment according to a customary method to remove oils applied on the filament surface. Then, the hanks were dipped in a solution consisting of 1 l of water, 16 g of stannous chloride and 20 ml of 36 percent by weight hydrochloric acid at room temperature for 3 minutes, and washed with water. The hanks were further dipped in a solution

Table 1—Continued

|   |                                        |                                          |
|---|----------------------------------------|------------------------------------------|
| 5 | Amount of plating solution             | 200 l                                    |
|   | pH                                     | 5.0                                      |
|   | Plating time                           | 20 minutes                               |
|   | Plating temperature                    | 80°C.                                    |
|   | Rate of projection of plating solution | varied within a range of 2 to 60 cm/sec. |

Table 2

| Rate of Projection of plating solution(cm/sec.) | Thickness of Plating Layer(μ)* |                       |                                | Reel-ability of hank | Adherence durability |
|-------------------------------------------------|--------------------------------|-----------------------|--------------------------------|----------------------|----------------------|
|                                                 | Outer portion of hank          | inner portion of hank | Thickness of Plating Layer(μ)* |                      |                      |
| 2(comparison)                                   | 0.14 – 0.22                    | 0.18 – 0.22           | 0.18 – 0.22                    | good                 | relatively good      |
| 10                                              | 0.21 – 0.23                    | 0.22 – 0.23           | 0.22 – 0.23                    | good                 | good                 |
| 40                                              | 0.23 – 0.25                    | 0.24 – 0.25           | 0.24 – 0.25                    | good                 | good                 |
| 60(comparison)                                  | 0.24 – 0.26                    | 0.24 – 0.26           | 0.24 – 0.26                    | poor                 | not good             |
| Dipping method (conventional method)            | 0.18 – 0.32                    | 0.16 – 0.27           | 0.16 – 0.27                    | extremely poor       | good                 |

\*Note: the thickness was measured with respect to 10 hanks.

consisting of 1 l of water incorporated with 0.3 g of palladium chloride and 3 m l of 36 percent by weight hydrochloric acid at room temperature for 3 minutes, and washed with water sufficiently. The thus activated hanks of polyvinyl alcohol filaments were hung on a cylinder provided with forwarding plates having 50 per 100 cm<sup>2</sup> of projection holes of a diameter of 3 mm and 10 partition plates. One hank was hung on one section formed between the two adjoining partition plates (the total length of the cylinder being 1 m and the diameter of the cylinder being 5 cm). The cylinder was rotated at a rate of 60 rotations per minute, and the direction of rotation was reversed every 2 minutes. The electroless nickel-plating was conducted under conditions indicated in Table 1. The state of the plating layer of the resulting plated filaments and the properties of the plated fibers are shown in Table 2.

For comparison, "Vinylon" filaments were activated under the same conditions as described above and the plating was conducted at 80°C. for 20 minutes by dipping the filaments in 200 l of a plating solution as indicated in Table 1. Results are also shown in Table 2.

25 The electroless plating was then conducted according to the process of this invention in the same manner as described above except that mercaptoimidazole was not incorporated in the plating solution (the rate of projection of the plating solution being 40 cm/sec). In about 3 minutes from the initiation of the plating reaction, the plating solution was blackened, and the plating ratio was only 12 percent.

30 On the other hand, where mercaptobenzimidazole was added as the stabilizer, even after 20 minutes had passed from the initiation of the plating reaction, no blackening of the plating solution was observed, and at this point the plating ratio was 21 percent.

35 The electroless plating was conducted according to the process of this invention under the same conditions as above by employing the stabilizers indicated in Table 40. In each run, even after 20 minutes from the initiation of the plating reaction (the rate of projection of the plating solution being 40 cm/sec.), the plating solution was not blackened. The plating ratios obtained after 20 minutes from the initiation of the plating reaction in each run are shown in Table 3.

Table 3

| Kind                                                                  | Stabilizer                                                  | Plating Ratio(%) |  |
|-----------------------------------------------------------------------|-------------------------------------------------------------|------------------|--|
|                                                                       |                                                             | Amount           |  |
| 0.2 % 2-mercaptopimidazoline solution in 0.2-N NaOH                   | 0.05 g of stabilizer solution per liter of plating solution | 25               |  |
| 0.2 % diphenyl guanidine solution in 0.2-N NaOH                       | 0.1 g of stabilizer solution per liter of plating solution  | 20               |  |
| mercaptobenzthiazole in the form of a solution in 0.2-N NaOH          | 2 mg of stabilizer compound per liter of plating solution   | 19               |  |
| tetramethyl thiuram disulfide in the form of a solution in 0.2-N NaOH | 5 mg of stabilizer compound per liter of plating solution   | 18               |  |

Table 1

| Composition of Plating Solution                      |
|------------------------------------------------------|
| Nickel sulfate                                       |
| Sodium hypophosphite                                 |
| Sodium citrate                                       |
| Sodium acetate                                       |
| 0.2 % Mercaptobenzimidazole solution (in 0.2-N NaOH) |
| Electroless Plating Conditions                       |

0.10 mole/l  
0.10 mole/l  
0.10 mole/l  
15 g/l  
0.1 g/l

## EXAMPLE 2

65 Ten hanks of 250 dr/36 f polyester filaments having a twist number of 150 turns per meter, each having a weight of 100 g, were reeled and deoiled according to customary procedures. Then, each hank was dipped in an aqueous solution of sodium hydroxide having a concentration of 100 g/l at 60°C. for 30 minutes and then washed with water to remove the alkali therefrom, following which the activation treatment was carried out

in the same manner as in Example 1. The hanks were hung on a cylinder having a total length of 1 m and a diameter of 5 cm and being provided with forwarding plates having 120 per 100 cm<sup>2</sup> of holes for projection of a plating solution having a diameter of 2 mm and 10 partition plates, one hank being hung on one section formed between the two adjoining partition plates. The cylinder was rotated at a rate of 60 rotations per minute and the rotation direction was reversed every two minutes. The plating was carried out at 80°C. for 20 minutes while projecting a plating solution having the same composition as illustrated in Table 1 of Example 1 at a flow rate of 30 cm/sec. The thickness of the plating layer was 0.23–0.25  $\mu$  in the outer portion of the hank and 0.24–0.26  $\mu$  in the interior portion. Thus, nickel-plated polyester filaments having a uniform plating layer were obtained.

### EXAMPLE 3

Five hanks of Vynylon spun yarn (count No. 20; monofilament denier = 1; degree of formalization = 30 mole percent), each having a weight of 100 g, were reeled and activated in the same manner as in Example 1. Then, the hanks were plated under the same conditions as shown in Table 1 of Example 1. Namely, the hanks were hung on a cylinder having a total length of 0.5 m and a diameter of 5 cm and being provided with forwarding plates having 76 per 100 cm<sup>2</sup> of projection holes of a diameter of 4 mm, one hank being hung on one section formed between the two adjoining partition plates. The electroless plating was effected at 87°C. for 25 minutes at a rate of projection of the plating solution of 25 cm/sec. The thickness of the resulting plating layer was 0.40–0.43  $\mu$  in the outer portion of the hank and 0.42–0.43  $\mu$  in the interior portion of the hank. Thus, a nickel-plated Vynylon spun yarn having a uniform plating layer was obtained. For comparison, a nickel-plated Vynylon spun yarn was prepared according to the conventional dipping plating method. In this comparative yarn, the thickness of the plating layer was 0.15–0.50  $\mu$  in the interior portion of the hank and 0.32–0.47  $\mu$  in the outer portion thereof.

### EXAMPLE 4

Ten hanks, each having a weight of 50 g, were reeled from 210 dr/24 nylon filaments having a twist number of 100 turns per meter and deoiled according to customary procedures. Then, the hanks were etched with a solution consisting of 1 l of water, 30 g of chromic anhydride, 150 g of concentrated sulfuric acid and 100 g of phosphoric acid at 40°C. for 3 minutes, and washed with water. Then the activation treatment was carried out in the same manner as described in Example 1, and the activated hanks were electrolessly plated by employing the same plating solution and plating apparatus as in Example 1, at 80°C. for 20 minutes while projecting the plating solution at a flow rate of 30 cm/sec. As a result, nickel-plated nylon filaments with a uniform plating having a thickness of 0.35–0.37  $\mu$  in the outer portion of the hank and 0.36–0.38  $\mu$  in the interior portion of the hank were obtained. Comparative nickel-plated nylon filaments prepared by the conventional dipping plating method had a plating layer with a thick-

ness of 0.25–0.39  $\mu$  in the outer portion of the hank and 0.19–0.32  $\mu$  in the interior portion of the hank.

### EXAMPLE 5

5 Ten hanks of the same Vynylon filaments as used in Example 1, each hank having a weight of 100 g, were subjected to the deoiling and activation treatments in the same manner as in Example 1. The activated hanks were then subjected to the electroless copper-plating 10 using the same plating apparatus as used in Example 1. The composition of the plating solution used and the plating conditions adopted are shown below:

| Composition of Plating Solution         |            |
|-----------------------------------------|------------|
| Copper sulfate                          | 17.5 g/l   |
| Rochelle salt                           | 85 g/l     |
| Sodium hydroxide                        | 25 g/l     |
| Formalin (37%)                          | 50 ml/l    |
| Mercaptobenzothiazole                   | 15 mg/l    |
| Electroless Plating Conditions          |            |
| Amount of plating solution              | 200 l      |
| Plating time                            | 15 minutes |
| Plating temperature                     | 25°C.      |
| Flow rate of projected plating solution | 35 cm/sec  |

25 As a result, copper-plated Vynylon filaments with a uniform plating layer having a thickness of 0.27–0.31  $\mu$  in the outer portion of the hank and 0.29–0.32  $\mu$  in the interior portion of the hank were obtained.

30 In comparative copper-plated Vynylon filaments obtained according to the conventional dipping method, unplated parts were observed here and there in the product, and it was impossible to obtain a plated product having a uniform plating.

### EXAMPLE 6

35 Five hanks of copper-plated Vynylon filaments prepared in Example 5 were hung on the same plating apparatus as used in Example 3, and the plating was conducted for 7 minutes under the same conditions as adopted in Example 3. A nickel plating was formed on the copper plating, and the nickel plating layer had a thickness of 0.15–0.17  $\mu$  in the outer portion of the hank and 0.16–0.18  $\mu$  in the interior portion of the hank. Thus, copper- and nickel-plated Vynylon filaments having a uniform plating were obtained.

### EXAMPLE 7

This Example illustrates that metal-plated filaments having a very excellent adherence durability can be obtained from polyvinyl alcohol filaments without conducting the etching treatment.

50 Polyvinyl alcohol filaments as used in Example 1 were subjected to the deoiling and activation treatments conducted in the same manner as in Example 1 without performing the etching treatment as in Example 1. The electroless plating was effected on the thus treated polyvinyl alcohol filaments under the same conditions as shown in Table 1 of Example 1 by employing the plating solution shown in Table 1 of Example 1.

55 Ten hanks, each having a weight of 100 g, were reeled from 250 dr/36 f polyester filaments having a twist number of 150 turns per meter, and were deoiled according to customary procedures. Then, they were dipped for 30 minutes in an aqueous solution of sodium hydroxide having a concentration of 20 g/l which was

Table 4

| Sample                     | untreated<br>(before<br>washing or<br>bending) | Electrical Resistance |     |     |                 |     |     |     |     |
|----------------------------|------------------------------------------------|-----------------------|-----|-----|-----------------|-----|-----|-----|-----|
|                            |                                                | washing (times)       |     |     | bending (times) |     |     |     |     |
|                            |                                                | 1                     | 5   | 10  | 10              | 20  | 50  | 100 | 200 |
| Vynylon<br>(250 dr/36 f)   | 30                                             | 35                    | 37  | 45  | 32              | 35  | 42  | 48  | 61  |
| Polyester<br>(250 dr/36 f) | 28                                             | 67                    | 120 | 350 | 55              | 182 | 490 | 571 | 797 |
| Nylon<br>(210 dr/34 f)     | 35                                             | 60                    | 116 | 290 | 43              | 121 | 216 | 364 | 572 |

15 maintained at 65°C. to effect the etching and washed with water to remove the alkali therefrom. Then, the hanks were activated in the same manner as in Example 1 and subjected to the electroless plating under the conditions indicated in Table 1 of Example 1 with use of the plating solution shown in Table 1 of Example 1.

10 Ten hanks, each having a weight of 50 g, were reeled from 210 dr/34 f nylon filaments, and were deoiled according to customary procedures. Then, the hanks were etched with a solution containing 1 l of water, 20 g of chromic anhydride, 300 g of concentrated sulfuric acid and 100 g of phosphoric acid and washed with water. Then, the hanks were subjected to the activation treatment conducted in the same manner as in Example 1, and the electroless plating was effected on the hanks under the same conditions as illustrated in Table 1 of Example 1 with use of the same plating solution as employed in Example 1.

15 Three kinds of the thus obtained metal-plated fibers were subjected to the following test to compare them to each other with respect to the durability of adherence between the metal layer and the filament. Each sample of the three kinds of the plated filaments was subjected to the bending test using a custom bending tester, and the electrical resistance was measured after the bending was conducted a prescribed number of times. The measured value was compared with the value of the electrical resistance of the sample before the bending test. Further, each sample was subjected to the washing test. One cycle of washing treatment comprised washing the sample with a rinsing liquor containing 1 g/l of a surface active agent (sold under the trademark "Monogen Uni" at 40°C. for 12.5 minutes by employing an ordinary electric washing machine. This washing treatment was repeated a prescribed number of times, and the electrical resistance was measured. The measured value was then compared with the value of the electrical resistance of the untreated sample. The smaller the increase of electrical resistance after the

20 15 washing or bending treatment, the better the durability of adherence between the plating layer and filaments. Results are shown in Table 4, where the electrical resistance is expressed in the unit of  $\Omega/3$  cm.

25 20 What we claim is:

30 25 1. A process for the production of metal-plated fibers by electrolessly plating pre-treated fibers, which comprises reeling the fibers into hanks, hanging the fibers in the hank form on a rotary cylinder having projection holes to suspend the fibers in the air, wherein the projection holes are from about 2 to about 5 mm in diameter and present in from about 25 to about 150 holes per 100  $\text{cm}^2$  of the cylinder surface, and wherein the fibers have a denier of from about 0.1 to about 15, allowing the fibers to move rotatively around the cylinder by rotation of the cylinder, projecting an electroless metal plating solution at a rate of 5 to 50 cm/sec from said projection holes against the rotatively moving fibers and thereby effecting the electroless plating of the fibers.

35 30 2. A process set forth in claim 1, wherein the fibers are polyvinyl alcohol fibers.

40 35 3. A process set forth in claim 1, wherein a plating layer which nickel or copper is formed on the fiber by the electroless plating.

45 40 4. A process set forth in claim 1, wherein the rate of projection of the plating solution is within a range of from 15 to 35 cm/sec.

50 45 5. A process set forth in claim 1, wherein the plating solution contains as a stabilizer at least one member selected from the group consisting of guanidines, thiourea derivatives, imidazolines, dithiocarbamic acid salts, thiurams, thiazoles and imidazoles.

55 50 6. A process set forth in claim 1, wherein a stabilizer is incorporated in the plating solution at a concentration of from 0.5 to 20 mg per liter of the plating solution.

\* \* \* \* \*

UNITED STATES PATENT OFFICE  
CERTIFICATE OF CORRECTION

Patent No. 3,864,148 Dated February 4, 1975

Inventor(s) Minoru Maekawa et al

It is certified that error appears in the above-identified patent and that said Letters Patent are hereby corrected as shown below:

In the Heading, correct the spelling of the Inventors' names to read as follows:

-- Minoru Maekawa; Hiroaki Morioka --

Signed and sealed this 8th day of April 1975.

(SEAL)

Attest:

RUTH C. MASON  
Attesting Officer

C. MARSHALL DANN  
Commissioner of Patents  
and Trademarks